

# UNITED STATES PATENT OFFICE.

JAMES F. O'BRIEN, OF CHICAGO, ILLINOIS.

## EXPLOSIVE.

1,037,300.

Specification of Letters Patent. Patented Sept. 3, 1912.

No Drawing.

Application filed January 11, 1912. Serial No. 670,645.

To all whom it may concern:

Be it known that I, JAMES F. O'BRIEN, a citizen of the United States, residing at Chicago, in the county of Cook, State of Illinois, have invented new and useful Improvements in Explosives, of which the following is a specification.

This invention relates to improvements in my chlorate of alkali metals and carbo-hydrate explosives; and it relates particularly to the provision of certain combinations and compounds for the purpose of simplifying the process of manufacture of the explosive.

The present invention follows along the general line of my explosives of the class described, and particularly follows along the line of my explosives as described in my applications for Letters Patent filed on September 5th, 1911, S. N. 647,474; September 20th, 1911, S. N. 650,373; October 24th, 1911, S. N. 656,529. Heretofore, particularly in the second application cited, my explosive has been so composed that the process of manufacture necessitated cooking or heating, some of the ingredients before they could be finally mixed to form the explosive. My present invention obviates this preliminary heating or cooking and enables me to directly form the explosive from the suitable ingredients without any preliminary processes other than grinding or finely dividing some of the ingredients.

In my former processes of the first two cited applications for the making of my explosive I had first cooked or heated the carbo-hydrate, adding water if necessary, so that a liquid was formed. This heated liquid was then mixed with the chlorate and other ingredients and came out as a plastic or semi-fluid mass. This mass was then divided into small particles of suitable size and shape and then dried. In order that each particle of the resultant explosive have its due proportions of the different ingredients, it is necessary that the mass be mixed in a liquid or semi-liquid condition; and the plastic mass resultant is very easily handled and divided into particles of any size and shape; and the moisture pervading the mass also greatly decreases any liability and tendency to accidental explosion. In the process of the third application cited the liquids of the molasses provided sufficient moisture for working the material. But the water present must subsequently be removed to form a dry product.

My new process, and the product thereof which is the subject matter of this application, attains all these desirable ends without the necessity of going through the various complications of the former processes, as will be seen from the following. As a basis for my new explosive I use preferably potassium chlorate; and the carbo-hydrate in the aggregate I have found, as stated in my former application, to best be about one third by weight of the amount of the chlorate. But, in this case, the carbo-hydrate is made up of two distinct substances, one liquid and the other solid; and typically I use a certain proportion of starch, preferably browned starch, and a certain proportion of molasses, preferably beet sugar molasses on account of its cheapness. The quantities of starch and molasses are so fixed that the carbo-hydrates in the starch and in the molasses will aggregate approximately one third of the amount of chlorate, by weight. For instance, if I use seventy five pounds of chlorate, then I typically use about twelve and one half pounds of the starch and about twenty five pounds of molasses. (This amount of molasses is based on the fact that in some cheap beet sugar molasses the amount of available carbo-hydrates is only about one half of the total molasses; in molasses where the carbo-hydrates run to a higher proportion, the total amount of molasses used would be proportionately smaller.) Allowing one half of the molasses for substances which will not enter into the re-action, substances other than carbo-hydrates, there is then in the compound above outlined a total of twenty five pounds of carbo-hydrates. This makes the ideal proportions of one part carbo-hydrate to three parts chlorate.

In connection with the above enumerated ingredients I have found a special efficiency in the combination of certain amounts of calcined clay, Portland cement, or like substances. I have found by repeated experiment that a small amount of potassium chlorid is left in solid state after the detonation of a mixture of chlorate and carbo-hydrate; and that increasing additions of some silicate material decrease the solid deposit. I have also found, with my general class of chlorate and carbo-hydrate explosives and particularly with one herein described, that an addition of the silicate material up to an amount of forty pounds (in the amount of

other substances given above) does not materially decrease the explosive energy of a given weight of explosive; that is specifically, that a pound of explosive containing the proportions 75 chlorate, 12½ starch, 25 molasses and 40 clay is approximately as strong as a pound containing the proportions 75 chlorate, 12½ starch and 25 molasses. From these facts I have arrived at the obvious conclusion that the silicate must carry with it some potential explosive energy to balance the energy of the chlorate and carbo-hydrate displaced. It seems that the aluminum silicates of calcined clay, or silicates of other materials such as Portland cement, react with potassium and chlorin to form other compounds and liberate oxygen. This active chemical action is in addition to the passive heat retaining quality in the clay or other material.

Calcined clay seems to give best results, carrying a high percentage of aluminum silicates. Portland cement is very conveniently used, however, as it can be readily obtained on the market in dry powdered form.

Any substance of a general character similar to these will give good results, it being apparent that the presence of silicates adds to the explosive energy. The other 30 pounds, such as calcium aluminates in Portland cement, are comparatively inert and act mainly as heat retainers. This action is also of no little importance, as the heat is thus more highly concentrated in the expanding gases generated by the explosion.

I have also found that the addition of a small amount of graphite or similar substance improves the mechanical and chemical qualities of the explosive. The grains 40 are smoothed exteriorly so as to reduce friction both in the operations of mixing the ingredients and handling the finished explosive. The carbon also enters into the chemical action of detonation.

It is in the process of manufacture of this particular explosive that it has one of the greatest utilities. As a preparatory measure it is only necessary that the chlorate and the starch be first finely divided. The chlorate, 50 starch, molasses, and clay or cement are then all mixed together in a suitable mixing machine; a suitable amount of graphite or similar substance is added and the mass is then divided and dried in any suitable manner.

(These operations are perfectly safe and may be performed indifferently). The starch is not necessarily liquefied, heated or dissolved preparatory to the mixing; the liquid molasses furnishes just the proportion 60 of moisture needed in the resultant mixture so that the mixture can be thoroughly agitated and be made homogeneous and so that it may be easily handled for division into small particles. The simplicity of this process over any other is readily ap-

parent; and the single machine for carrying on the process is equally simple. And what effects this simplicity is the provision, in combination with the other ingredients, of the carbo-hydrates partly in solid form and partly in liquid form—specifically partly as starch or sugar and partly as molasses. The molasses and silicates lend cheapness to the whole compound; whereas the combination of the molasses and the other solid carbo-hydrates lends cheapness to the process of manufacture.

In its finished state, the above described explosive is possessed of many advantages. All danger of accidental explosion is totally avoided. (Heretofore chlorate explosives have been considered extremely unsafe). Unless confined, a mass cannot be detonated by flame, vibration or shock or violent percussion. It will only detonate when confined and subjected to flame. No change, chemical or physical takes place when the explosive is exposed for long periods. It is smokeless and leaves no noxious gases or fumes. Its strength is equal to 60%—80% dynamite. All these qualities make my explosive highly useful when a powerful detonator is desired which is absolutely safe and comparatively inexpensive.

A special advantage inheres in the use of 95 Portland cement, in that it quickly absorbs the moisture in the mixture and causes rapid solidification. The molasses being non-deliquescent, very rapid setting can thus be obtained.

Having described my invention, I claim:

1. An explosive, comprising potassium chlorate, starch, molasses, and a silico-aluminous substance.

2. An explosive, consisting of approximately a chlorate seventy five pounds, a solid carbo-hydrate twelve and one half pounds; a carbo-hydrate in solution twenty five pounds, and a silico-aluminous substance less than forty pounds.

3. An explosive, consisting of a chlorate, a solid carbo-hydrate, a carbo-hydrate in solution, and Portland cement.

4. An explosive, consisting of approximately a chlorate seventy five pounds; a solid carbo-hydrate twelve and one half pounds, a carbo-hydrate in solution twenty five pounds, and Portland cement less than forty pounds.

5. An explosive, comprising starch, molasses, a chlorate of an alkali metal, and a silico-aluminous material.

6. An explosive, comprising approximately a chlorate of an alkali metal seventy five parts by weight, starch twelve and one half parts, molasses twenty five parts, and a silico-aluminous substance less than forty parts.

7. An explosive, comprising approximately potassium chlorate seventy-five parts

by weight, starch twelve and one half parts, molasses twenty five parts, and a silico-aluminous substance less than forty parts.

8. An explosive, consisting of starch, molasses, a chlorate of an alkali metal, and Portland cement.

9. An explosive, consisting of potassium chlorate, seventy-five parts by weight, starch twelve and one half parts, molasses twenty-

five parts, and Portland cement less than 10 approximately forty parts.

In witness that I claim the foregoing I have hereunto subscribed my name this 3d day of January 1912.

JAMES F. O'BRIEN.

Witnesses:

JAMES T. BARKELEW,  
ELWOOD H. BARKELEW.

Copies of this patent may be obtained for five cents each, by addressing the "Commissioner of Patents,  
Washington, D. C."